

## UNITED STATES PATENT OFFICE

PHILIPPE BRANDT, OF MULHOUSE, FRANCE, AND KARL GLENZ, OF BASEL, SWITZERLAND, ASSIGNORS TO THE FIRM DURAND & HUGUENIN S. A., OF BASEL, SWITZERLAND

## PROCESS FOR OBTAINING FAST DYEINGS AND PRINTS WITH VAT DYESTUFFS

No Drawing. Application filed December 14, 1929, Serial No. 414,243, and in Germany December 22, 1928.

From the ester salts of leuco vat dyestuffs, known as indigosols, obtained according to the process of the U. S. Letters Patent No. 1,448,251, or other processes, the original vat dyestuff can easily be re-formed by acid oxidation.

This easy re-formation of insoluble vat dyestuffs from such water soluble ester salts allows the application of the latter for dyeing and printing textile fibres and other materials (see U. S. Letters Patent No. 1,575,958).

This fundamental dyeing process has been modified in various directions (see U. S. Letters Patent No. 1,645,925 and U. S. patent application Ser. No. 202,473, filed June 29, 1927). Thus, the re-formation of the vat dyestuff on a fibre, or in other words, the dyeing can be effected by means of an ester salt with a suitable oxidizing agent by a steaming operation in an analogous manner to what is the case with dyeings of aniline black.

This steam developing process, although modified and improved in different ways (see U. S. Patent No. 1,747,107, is not yet quite satisfactory. What should be aimed at is a complete re-formation of the vat colour on the fibre, avoiding, however, any other disturbing reaction. This can only be attained if oxidizing agents, steam conditions, etc. are strictly adapted to the oxidizing conditions required for the development of a specific ester salt, so that on the one hand the ester salt is completely oxidized to the vat colour, and on the other hand, for instance in the case of sensitive dyestuffs, no over-oxidation can take place. In order to obtain satisfactory results, therefore, the kind and quantity of the oxidizing agent, as well as the other conditions for any individual case, must be selected accurately; but thereby the possibility of application of the process is prejudiced.

It has now been found that this steam developing process for ester salts of leuco vat dyestuffs can be improved if certain materials are used which play the part of buffer-materials, i. e. which admit the oxidizing effect necessary for the development of the

dyeing, but which render innoxious any possible excess of oxidizing agent.

Thus, it is possible to use a certain excess of oxidizing agent so that, on the one hand, in spite of bad steaming conditions which do not allow of a good use being made of the oxidizing agents, complete development can take place, and on the other hand, with good steaming conditions, an over-oxidation can be avoided.

Substances which meet the present case are aromatic amino-bodies containing a negative salt-forming group such as a sulphonate group or a carboxylic group. Such substances are therefore sulphonate acids or carboxylic acids respectively their salts of aniline, of the alkylanilines, of the homologues of these compounds, also of the naphthylamines etc. These are bodies which are soluble in water, which are not volatile under conditions of steaming and which under the present circumstances do not form any disturbing oxidation colours.

In the present process the said products can either be added to the printing pastes or to the dry ester salts.

The effect of the above mentioned additions could not be foreseen.

The process is explained by the following examples:

(I) Make up the following printing colour:

|                                                                                                                                      | Parts |
|--------------------------------------------------------------------------------------------------------------------------------------|-------|
| Ester salt of the leuco vat dyestuff 2- $\beta$ - $\alpha$ -naphthindol-2'-p-chloroanthra-cene-indigo containing 55% of vat dyestuff | 85    |
| Sodium sulphinate                                                                                                                    | 7.2   |
| Water                                                                                                                                | 4.2   |
| Diethyltartrate                                                                                                                      | 18    |
| Gum tragacanth thickening                                                                                                            | 8     |
| Solution of sodium chlorate (10%)                                                                                                    | 90    |
| Solution of vanadate of ammonia (1%)                                                                                                 | 50.6  |
| Ammonia                                                                                                                              | 12    |
|                                                                                                                                      | 4     |
|                                                                                                                                      | 1     |
|                                                                                                                                      | 95    |
|                                                                                                                                      | 100   |

Print on cotton, steam for 10 minutes in the rapid ager, soap for 1 minute at the boil, and wash. A well developed black dyeing is obtained.

If in this printing paste the sodium sulphanilate is omitted or is replaced by an indifferent substance, such as for instance, sodium sulphate, then, owing to overoxidation, weak, dull, grey-green tints result.

5 (II) Make up the following printing colour:

|                                                                                                                                                                              | Parts |
|------------------------------------------------------------------------------------------------------------------------------------------------------------------------------|-------|
| 10 Ester salt of the leuco vat dyestuff obtained from 5:7-dibrom-isatin- $\alpha$ -chloride with $\alpha$ -anthol (see Colour Index No. 1203) containing 65% of vat dyestuff |       |
| 15 Sodium salt of diethylaniline metasulphonic acid                                                                                                                          |       |
| 20 Water                                                                                                                                                                     |       |
| 25 Gum tragacanth thickening                                                                                                                                                 |       |
| 30 Solution of sodium chlorate (10%)                                                                                                                                         |       |
| 35 Solution of sulphocyanide of ammonia (1:1)                                                                                                                                |       |
| 40 Solution of vanadate of ammonia (1%)                                                                                                                                      |       |
|                                                                                                                                                                              | 100   |

Print on cotton, steam for 10 minutes in the rapid ager, soap and wash. Level and well developed dyeings are obtained.

Without the addition of the sodium salt of diethylaniline meta-sulphonic acid, still useful, but bad, over-oxidized dyeings are obtained in accordance with the steaming conditions.

(III) Make up the following two printing colours *a* and *b*:

|                                               | Parts | <i>a</i> | <i>b</i> |
|-----------------------------------------------|-------|----------|----------|
| 35 Ester salt of leuco indigo                 | 4.6   | 4.6      |          |
| 40 Sodium sulphanilate                        | 3.4   | 3.4      |          |
| 45 Monoethylglycol                            | 5     | —        |          |
| 50 Diethyltartrate                            | 2     | —        |          |
| 55 Water                                      | 14    | 14       |          |
| 60 Gum tragacanth thickening                  | 55    | 58       |          |
| 65 Solution of sulphocyanide of ammonia (1:1) | —     | 3        |          |
| 70 Solution of sodium chlorate (10%)          | 4     | 8        |          |
| 75 Solution of vanadate of ammonia (1%)       | 10    | 8        |          |
| 80 Ammonia                                    | 2     | 1        |          |
|                                               | 100   | 100      |          |

Print on cotton, steam for 10 minutes, then soap and wash. In both instances well developed reddish-blue tints are obtained. If, however, the sodium sulphanilate is omitted, or if this material is replaced by an indifferent one, owing to over-oxidation only weak, greenish-blue tints are obtained.

When using the other indigosols according to the present process, advantageous results are also obtained.

In place of the additions mentioned in the above examples, other substances, such as for instance monoethyl-aniline-meta-or-para-sulphonic acid, mono- or dimethyl-aniline-meta-

or-para-sulphonic acid, naphthylamine-sulphonic acids, aminobenzoic acids, etc., or their salts, etc., can be used with a similar effect.

What we claim is:—

1. A process for dyeing and printing with vat dyestuffs by applying to the goods an ester salt of a leuco vat dyestuff, a suitable oxidizing agent and a substance capable of forming acid when heated, and engaging by a steaming operation the acid oxidizing action necessary for the development of the dyeing, this process being characterized by the fact that it is conducted in the presence of an aromatic aminobody containing a negative salt-forming group. 70

2. A process for dyeing and printing with vat dyestuffs by applying to the goods an ester salt of a leuco vat dyestuff, a suitable oxidizing agent and a substance capable of forming acid when heated, and engaging by a steaming operation the acid oxidizing action necessary for the development of the dyeing, this process being characterized by the fact that it is conducted in the presence of an aromatic aminobody with a negative 80 salt-forming group, used in form of a salt. 90

3. A process for dyeing and printing with vat dyestuffs by applying to the goods an ester salt of a leuco vat dyestuff, a suitable oxidizing agent and a substance capable of forming acid when heated, and engaging by a steaming operation the acid oxidizing action necessary for the development of the dyeing, this process being characterized by the fact that it is conducted in the presence of an aromatic amino sulpho body. 100

4. A process for dyeing and printing with vat dyestuffs by applying to the goods an ester salt of a leuco vat dyestuff, a suitable oxidizing agent and a substance capable of forming acid when heated, and engaging by a steaming operation the acid oxidizing action necessary for the development of the dyeing, this process being characterized by the fact that it is conducted in the presence of an aromatic amino sulpho body used in 105 form of a salt. 110

5. A process for dyeing and printing with vat dyestuffs by applying to the goods an ester salt of a leuco vat dyestuff, a suitable oxidizing agent and a substance capable of forming acid when heated, and engaging by a steaming operation the acid oxidizing action necessary for the development of the dyeing, this process being characterized by the fact that it is conducted in the presence of sodium sulphanilate. 115 120

In witness whereof we have hereunto signed our name this 3rd day of December, 1929.

PHILIPPE BRANDT.  
KARL GLENZ.